

1

3,313,732  
CYCLIC KETO ESTERS AND LUBRICANTS  
CONTAINING THEM

Keith Coupland and John Pennington, Hull, and Sidney John Branch, Hornsea, England, assignors to The Distillers Company Limited, Edinburgh, Scotland, a British company  
No Drawing. Filed Nov. 12, 1964, Ser. No. 410,772  
Claims priority, application Great Britain, Nov. 28, 1963, 46,968/63; Apr. 1, 1964, 13,512/64  
1 Claim. (Cl. 252—57)

This invention relates to synthetic lubricants and in particular to synthetic lubricant bases.

Synthetic lubricant bases may comprise, for example, esters such as diethyl and dinonyl sebacates. In order to fulfill completely the requirements of a practical lubricant composition, various additives are customarily added to the base, which normally constitutes at least 60% and more, usually at least 90% by weight of the lubricant composition. Such additives include antioxidants (for instance phenothiazine or diethyl phenothiazine); viscosity index improvers (for instance polymethacrylates or polyglycolethers); load carrying additives (for instance trityl phosphate or trixylyl phosphate), metal de-activators and anti-corrosion agents. The nature and quantity of such additives are varied as required for any particular lubricant composition to fulfill specific desiderata.

The present invention provides a synthetic lubricant base containing at least one keto-ester of formula:



or



wherein  $\text{R}^1$ ,  $\text{R}^2$ ,  $\text{R}^3$  and  $\text{R}^4$  are the same or different alkyl groups, each of preferably from 4 to 16 carbon atoms, and  $\text{R}^5$  is an alkyl group such as the methyl group.

These compounds may, with advantage, be used as synthetic lubricant bases in admixture with a compound having at least two ester groupings in the molecule, such as the alkyl esters of organic dicarboxylic acids and monocarboxylic acid esters of polyalcohols. It is contemplated that halogen-substituted esters are also useful as compounds having at least two ester groupings in the molecule.

2

Accordingly the present invention further provides a synthetic lubricant base composition comprising at least one keto-ester of formula



or



wherein  $\text{R}^1$ ,  $\text{R}^2$ ,  $\text{R}^3$ ,  $\text{R}^4$  and  $\text{R}^5$  are as hereinbefore defined, in admixture with a compound having at least two ester groupings in the molecule.

Suitable compounds having at least two ester groupings in the molecule include diethyl sebacate, dinonyl sebacate, esters of trimethylol propane such as trimethylol propane tricaprylate and esters of pentaerythritol.

The proportions of keto-ester and compound having at least two ester groupings in the molecule in the synthetic lubricant bases of the invention will, naturally, vary within wide limits according to the requirements for the particular base to be formulated. Suitable proportions are within the range 85% to 10%, especially 70% to 25%, particularly 30-35% of keto-ester by weight of the total base.

The keto-esters employed in the synthetic lubricant bases of the invention can be prepared for example by cyanoethylation of the appropriate cycloalkanone or alkyl-substituted cycloalkanone, followed by hydrolysis of the resulting tetra- or tri-nitrile, to give the corresponding acid. Such a reaction is described for specific compounds in J. Amer. Chem. Soc., 64, 2850-2858. The acid is then esterified with a small excess of the appropriate alcohol together with entrainer and an esterification catalyst. The reaction conditions are selected to give esterification temperatures within the range of 90° C. to 180° C., preferably between 120° C. and 160° C. High temperatures within the quoted ranges do not significantly affect ester yield or quality, but are useful in promoting satisfactory reaction rates. The entrainer may be for example benzene, toluene, cyclohexane or any other hydrocarbon capable of forming a binary azeotrope with water. The alcohol used may be any saturated aliphatic or cycloaliphatic alcohol having from 1 to 16, preferably 4 to 16 carbon atoms. The excess of alcohol employed in the esterification is suitably at least 2% and preferably 3-13% based on the weight of acid. Any of the known esterification catalysts may be used, but sulphuric acid is preferred. The amount of catalyst used depends on the purity of the acid to be esterified, but generally 0.05 to 1.0% w./w. sulphuric acid based on the total esterification charge is satisfactory.

The crude ester is generally dark brown in colour and can be decolourized by ozone, potassium permanganate, bromine or sodium hypochlorite, but it is preferred to wash the crude ester with  $2 \times \frac{1}{4}$  volumes of aqueous 10% w./v. sodium hydroxide solution,  $1 \times \frac{1}{4}$  volume of aqueous 10% w./v. sodium chloride solution and  $1 \times \frac{1}{4}$  volume of distilled water. Sodium hydroxide solutions of less than 5% w./v. are less effective decolourants and significant improvements are not obtained by the use of sodium hydroxide solutions of greater concentration than 10% w./v.

Some of the keto-esters of which the preparation has been described above are new compounds. Accordingly the present invention still further provides keto-esters of formula



or



wherein  $\text{R}^1$ ,  $\text{R}^2$ ,  $\text{R}^3$ , and  $\text{R}^5$  have the meanings ascribed above.

Lubricant bases of this invention have in general satisfactory properties for use in turbine engine lubricants.

It may be seen from the table that keto-esters of this invention have very good oxidative stability and thermal volatility and possess adequate viscosity at 210° F., and adequate low temperature fluidity.

#### Example 7

A mixture of 70% of the keto-ester of Example 3 with 30% of diethyl sebacate was evaluated according to the above procedure. It had the following properties:

|    |                                         |     |
|----|-----------------------------------------|-----|
| 10 | Oxidative stability, percent w./w. loss | 26  |
|    | Thermal volatility, percent w./w. loss  | 3   |
|    | Viscosity increase                      | Nil |
|    | Viscosity at 210° F., centistokes       | 8.6 |
| 15 | Pour point, ° F.                        | -65 |

#### Example 8

A mixture of 55% of the keto-ester of Example 3 with 45% of dinonyl sebacate was evaluated according to the procedure described in Example 1 in respect of oxidative stability, viscosity and pour point. The results were as follows:

|    |                                          |           |
|----|------------------------------------------|-----------|
| 20 | Oxidative stability, percent weight loss | 35        |
|    | Viscosity at 210° F., centistokes        | 7.8       |
| 25 | Viscosity at 100° F., centistokes        | 52.1      |
|    | Pour point, ° F.                         | Below -60 |

The normal volatility of this material was assessed in similar manner to that used in Example 1 but under more severe conditions, since the temperature of the ester was maintained at 340° C. The thermal properties of this material at this temperature are shown in Table 2, together with the properties of dinonyl sebacate.

TABLE 2

| Ester                             | Thermal volatility (340° C.) |                        | After test           |                   |
|-----------------------------------|------------------------------|------------------------|----------------------|-------------------|
|                                   | Weight loss, percent         | Viscosity increase     | Acid No., Mg. KOH/g. | Appearance        |
| Dinonyl sebacate                  | 36                           | Material solidified... | 238                  | Solid.            |
| 55% Ester 4, 45% dinonyl sebacate | 27                           | Small...               | 36                   | Slight darkening. |

#### Example 9

45 A mixture of 45% of the keto-ester of Example 4 with 55% of diethyl sebacate, with the addition of 3% of a polymeric methacrylate viscosity index improver had the following properties:

|    |                                          |           |
|----|------------------------------------------|-----------|
| 50 | Oxidative stability, percent weight loss | 51        |
|    | Viscosity at 210° F., centistokes        | 7.6       |
|    | Viscosity at 100° F., centistokes        | 39.6      |
|    | Pour point, ° F.                         | Below -60 |

#### Example 10

55 A mixture of 65% of the keto-ester of Example 4 with 35% of trimethylol propane tricaprylate had the following properties:

|    |                                          |      |
|----|------------------------------------------|------|
| 60 | Oxidative stability, percent weight loss | 26   |
|    | Viscosity at 210° F., centistokes        | 8.0  |
|    | Viscosity at 100° F., centistokes        | 52.2 |
|    | Pour point, ° F.                         | -60  |

TABLE 1

| Example/Comparison Number | Ester                                                                                             | Oxidative Stability Weight loss (percent) | Thermal volatility    |                    | Viscosity at 210° F. Centistokes | Pour point, ° F. |
|---------------------------|---------------------------------------------------------------------------------------------------|-------------------------------------------|-----------------------|--------------------|----------------------------------|------------------|
|                           |                                                                                                   |                                           | Weight loss (percent) | Viscosity increase |                                  |                  |
| A                         | Dinonyl sebacate                                                                                  | 79                                        | 12                    | 7                  | 4.6                              | -80              |
| 1                         | Esters of this invention:<br>$\text{R}^1 = \text{R}^2 = \text{R}^3 = \text{R}^4 = \text{n-Butyl}$ | 15                                        | 15                    | Nil                | 10.6                             | -35              |
| 2                         | $\text{R}^1, \text{R}^2, \text{R}^3$ and $\text{R}^4$ mixed $\text{C}_7, \text{C}_9$ alkyl        | 15                                        | 6                     | Nil                | 17.0                             | -15              |
| 3                         | $\text{R}^1 = \text{R}^2 = \text{R}^3 = \text{R}^4 = 2\text{-ethylhexyl}$                         | 16                                        | 6                     | Nil                | 14.4                             | -20              |
| 4                         | $\text{R}^1, \text{R}^2, \text{R}^3$ and $\text{R}^4$ mixed $\text{C}_8, \text{C}_{10}$ alkyl     | 14                                        | 6                     | Nil                | 12.0                             | -30              |
| 5                         | $\text{R}^1, \text{R}^2, \text{R}^3 = \text{n-butyl}$ , $\text{R}^4 = \text{methyl}$              | 28                                        |                       |                    |                                  | -40              |
| 6                         | 1,1,3,3 tetra(n-butyl- $\beta$ -propionate) cyclopentan-2-one                                     | 6                                         |                       |                    |                                  |                  |

## Example 11

A mixture of 33% of the keto-ester of Example 1 with 66% of trimethylolethane tricaprylate had the following properties:

|                                                    |      |
|----------------------------------------------------|------|
| Oxidative stability (500° F.), percent weight loss | 20   |
| Viscosity at 210° F., centistokes                  | 5.3  |
| Viscosity at 100° F., centistokes                  | 30.6 |
| Pour point, ° F.                                   | —65  |

We claim:

A synthetic lubricant composition wherein the lubricant base comprises at least one keto-ester of formula selected from the group consisting of



and



wherein  $\text{R}^1$ ,  $\text{R}^2$ ,  $\text{R}^3$ ,  $\text{R}^4$  and  $\text{R}^5$  are alkyl groups, and wherein said lubricant base also contains a compound having at least 2 ester groupings in the molecule, said compound being selected from the group consisting of dinonyl sebacate, diotetyl sebacate and trimethylolethane tricaprylate, the keto-ester constituting from 85% to 10% of the weight of the lubricant base.

## References Cited by the Examiner

## UNITED STATES PATENTS

- |           |         |                 |             |
|-----------|---------|-----------------|-------------|
| 2,386,736 | 10/1945 | Bruson          | 260—465.4 X |
| 2,403,570 | 7/1946  | Weist et al.    | 260—464     |
| 2,460,536 | 2/1949  | Rogers          | 260—465.4 X |
| 3,057,815 | 10/1962 | Bartlett et al. | 252—57 X    |

## FOREIGN PATENTS

- |    |         |        |         |
|----|---------|--------|---------|
| 25 | 638,161 | 3/1962 | Canada. |
|----|---------|--------|---------|

## OTHER REFERENCES

Barnes et al.: "Lubricating Engineering," August 1957, pages 454—458.

- |    |                                    |
|----|------------------------------------|
| 30 | DANIEL E. WYMAN, Primary Examiner. |
|    | W. H. CANNON, Assistant Examiner.  |